

Aug. 12, 1952

J. A. ROY ET AL

2,607,014

ELECTRIC GASEOUS DISCHARGE DEVICE

Filed Nov. 8, 1947



JOSEPH ARTHUR ROY,  
ROBERT S. IVES,

INVENTORS

BY *Landane Brown*

ATTORNEY

UNITED STATES PATENT OFFICE

2,607,014

## ELECTRIC GASEOUS DISCHARGE DEVICE

**Joseph Arthur Roy, Danvers, and Robert S. Ives,  
Topsfield, Mass., assignors to Sylvania Electric  
Products Inc., Salem, Mass., a corporation of  
Massachusetts**

Application November 8, 1947, Serial No. 784,806

**2 Claims. (Cl. 313—109)**

1

This invention relates to electric gaseous discharge devices and more particularly to a means for improving the maintenance of the radiant flux output of said devices during life.

In the manufacture of electric gaseous discharge devices, such as fluorescent lamps and germicidal lamps, for example, one of the primary objects is to make a device which will be characterized by a high radiant flux output throughout its life. In the case of devices emitting visible light, the radiant flux is usually expressed in terms of lumens per watt. The ideal device would be one which suffered no loss in radiant flux output throughout its life. However, during the course of their lives, electric gaseous discharge devices suffer a loss in their radiant flux output. In some cases the loss is greater than in others. In some cases a substantial loss is suffered early in life and the loss increases as the life expectancy of the device is approached.

An object of this invention is to provide means for reducing the loss in radiant flux output during the life of electric gaseous discharge devices.

Another object is to provide means for increasing the brightness or lumens per watt output of a fluorescent lamp during life.

In our co-pending application, Serial No. 680,527, filed June 29, 1946, now abandoned, of which this application is a continuation in part we pointed out that the addition of small quantities of  $Sb_2O_3$  to a suspension of luminescent material adapted to be used as a coating for fluorescent material adapted to be used as a coating for fluorescent lamps aids considerably in maintaining a high L. P. W. output throughout the life of the lamp. We also indicated that this addition of  $Sb_2O_3$  to the luminescent material suspension was particularly satisfactory when zinc silicate, zinc beryllium silicate, and/or magnesium tungstate was the luminescent material used.

The addition of a small quantity of antimony in the form of the free metal or certain of its compounds, such as the oxides for example, is beneficial not only to fluorescent lamps but to other types of electric gaseous discharge devices, particularly when the envelope is a soda-lime or borosilicate glass. The effect on the maintenance of the radiant flux output of these devices is particularly beneficial when the devices contain a metal vapor, such as mercury.

In the case of fluorescent lamps, the envelope of which is usually soda-lime glass, antimony may be added to the finished phosphor, not only in the form of the trioxide but the free metal.

7,014,000 Serial No. 1,038,000 filed 10/20/46, issued 10/20/47  
**DISCHARGE DEVICE** *John M. Collier, John F. Lusk, John C. Lusk, and Robert S. Ives, inventors, to Sylvania Electric Products Incorporated, a corporation of Mass., a corporation of*  
2,147,313 Serial No. 784,806 filed 10/20/46, issued 10/20/47  
**CL. 313—109** *John M. Collier, John F. Lusk, John C. Lusk, and Robert S. Ives, inventors, to Sylvania Products Incorporated, a corporation of Mass., a corporation of*  
2. *2*  
the pentoxide, and many other antimony compounds may also be used with beneficial results. The lumen maintenance and the brightness during life of fluorescent lamps may also be increased by providing the inner wall of the lamp envelope with a surface containing antimony or certain of its compounds before the fluorescent material is applied thereto. If desired, antimony or its oxides may be added to the raw material mixture of some fluorescent materials before they are fired with beneficial results. However, further additions to the finished phosphor generally increase the beneficial effect on the L. P. W. maintenance and the brightness during life.  
15. *In the case of other types of electric gaseous discharge devices which do not have a fluorescent coating, such as germicidal lamps, the inner wall of the lamp envelope, which is normally a borosilicate glass, is provided with a surface high in antimony content. This may be accomplished, for example by mixing the free metal or the antimony compound selected with a suitable lacquer, such as nitrocellulose for example, and applying this mixture to the inner wall of the lamp envelope. The lamp envelope is then heated to a temperature sufficient to burn off the lacquer.*  
30. *The quantity of antimony or its compounds necessary to obtain a beneficial effect on the maintenance of the radiant flux output of an electric gaseous discharge device is quite small. For example, in the case of fluorescent lamps, the L. P. W. maintenance and the brightness during life is improved when the quantity of antimony or its compound which is added during manufacture is greater than .005% and less than 1%. The addition of more than 1% tends to depress the brightness of the lamp early in life and from a practical commercial viewpoint this is not desirable. When the amount of antimony or a compound thereof which is added is kept below 0.1%, the discoloration which normally appears on the fluorescent coating on the lamp envelope after the lamp has burned several hundred hours is not increased. However, the addition of more than 0.1% tends to cause serious discoloration near the ends of the lamp envelope and, in the absence of some means for correcting this condition, the amount of antimony or a compound thereof which is added should not be more than 0.1%. With respect to discoloration, therefore, the amount of antimony or a compound thereof which is added is critical. The preferred addition, in view of these several factors, is about .05%.*

fluorescent lamp. The lamp comprises an elongated tubular glass envelope 1 which is provided on its inner wall with a coating of fluorescent material 2. The fluorescent material is applied by suspending it in a suitable lacquer and causing it to flow over the wall of the lamp envelope. After this suspension has dried, the lamp envelope is heated in an oxidizing atmosphere at a temperature high enough to burn off the lacquer, such as between about 450° C. to about 550° C. Stems 3 are sealed in the ends of the envelope. Lead wires 4 are sealed in the stems and the inner ends thereof serve as supports for filamentary electrodes 5 which are provided with a coating of an electron emissive material, such as the alkaline earth oxides, for example, as shown in the Lowry Patent 2,258,158. The lamp envelope is then exhausted and provided with a filling of an inert gas, such as argon, at low pressure, of the order of a few millimeters, such as 20 three millimeters for example. A small quantity of mercury 6 is also disposed within the envelope. During exhaust, the lamp is heated at a temperature below that at which the lamp envelope is baked to burn off the lacquer. The lamp is 25 usually operated at a mercury vapor pressure of between 1 to 20 microns.

Several of the examples below indicate the beneficial effect which the addition of a small quantity of antimony or certain of its compounds to a finished phosphor before it is applied to the wall of the lamp envelope has on the L. P. W. maintenance and the brightness during life of fluorescent lamps. In these examples, the antimony or a compound thereof, for convenience, has been added directly to the suspension of fluorescent material with which the lamp envelope is coated. However, the antimony or a compound thereof may be mixed with the powdered finished phosphor before it is put in suspension, or it may be mixed in a suitable medium and this mixture added to the suspension without departing from the spirit of the invention. The suspension of the finished phosphor and antimony or a compound thereof should be milled to insure thorough dispersion of the antimony or the compound used. This will give the antimony a particle size about the same as that of the finished phosphor.

EXAMPLE I.—ZINC BERYLLIUM MANGANESE SILICATE

The zinc beryllium manganese silicate may be prepared by mixing about 585 grams of ZnO, about 20 grams of BeO, about 56 grams of an activator, MnCO<sub>3</sub>, about 315 grams of silicic acid (containing about 277 grams of SiO<sub>2</sub>) and 0.6 grams of a fluxing agent, ZnF<sub>2</sub>. This mixture is fired at about 2230° to 2260° F. for from 4 to 6 hours to give a particle size of about 2.0 to 2.5 microns. The fired material is then ball milled, and suspended in a suitable lacquer such as nitrocellulose and the viscosity thereof may be adjusted by the addition of a solvent such as amyl acetate or butyl acetate. A small quantity of a plasticizer such as di-methyl-phthalate may also be added.

To this suspension a small quantity of powdered Sb<sub>2</sub>O<sub>5</sub> is added. The Sb<sub>2</sub>O<sub>5</sub> may be milled with a small amount of the same lacquer in which the luminescent material is suspended and then mixed with the luminescent material suspension or it may be added directly. In either case, the suspension of luminescent material with the Sb<sub>2</sub>O<sub>5</sub> added should be milled to insure thorough dispersion. This suspension is then applied to the lamp

bulb to form a coating which is dried, then baked. Electrodes are then sealed in the ends of the bulb and the lamp is processed in the conventional manner.

5 The table below shows the L. P. W. readings at various hours in life of the 40 watt lamps tested. Some of the lamps had .15% Sb<sub>2</sub>O<sub>5</sub> added to the fluorescent material suspension, and others had .30% added, both percentages being by weight of the finished phosphor.

LUMENS PER WATT

|                                           | 0<br>Hrs. | 100<br>Hrs. | 300<br>Hrs. | 500<br>Hrs. | 875<br>Hrs. | 1500<br>Hrs. |
|-------------------------------------------|-----------|-------------|-------------|-------------|-------------|--------------|
| 0% Sb <sub>2</sub> O <sub>5</sub> .....   | 61.0      | 54.8        | 51.4        | 49.6        | 47.2        | 45.8         |
| .15% Sb <sub>2</sub> O <sub>5</sub> ..... | 63.6      | 58.0        | 55.4        | 54.0        | 51.8        | 49.8         |
| .30% Sb <sub>2</sub> O <sub>5</sub> ..... | 58.4      | 55.2        | 53.4        | 52.2        | 50.4        | 48.8         |

Thus it may be seen from the above tabular data that the addition of Sb<sub>2</sub>O<sub>5</sub> to the suspension of luminescent material effects a substantial decrease in the rate of loss of lumens-per-watt output and an increase in the brightness of a fluorescent lamp during its life.

EXAMPLE II.—ZINC BERYLLIUM MANGANESE SILICATE

In this test the same raw materials in substantially the same proportions were used, except that about .08% PbO and about .001% As<sub>2</sub>O<sub>3</sub> by weight of the zinc oxide were added to the raw material mixture. The addition of small quantities of lead and arsenic to the raw materials used in making luminescent zinc silicates usually enhances the L. P. W. maintenance and brightness of fluorescent lamps. The mixture of raw materials was fired for from 3 to 6 hours at about 2210° F., ball-milled, and then fired again for about the same time and at about the same temperature. The particle size of the finished phosphor was about 3.75 microns. The suspension of the finished phosphor was prepared in substantially the same way as in Example I and about .05% Sb<sub>2</sub>O<sub>5</sub> by weight of the finished phosphor was added thereto. The effect which the addition of .05% Sb<sub>2</sub>O<sub>5</sub> had on the lumen maintenance and brightness of 40 watt lamps coated with this suspension is indicated in the following table:

LUMENS PER WATT

|                                           | 0<br>Hrs. | 100<br>Hrs. | 300<br>Hrs. | 500<br>Hrs. |
|-------------------------------------------|-----------|-------------|-------------|-------------|
| 0% Sb <sub>2</sub> O <sub>5</sub> .....   | 67.0      | 62.8        | 59.4        | 55.8        |
| .05% Sb <sub>2</sub> O <sub>5</sub> ..... | 66.0      | 64.4        | 61.4        | 61.4        |

65 This test indicates that a still further improvement in lumen maintenance and brightness can be obtained, in addition to that obtained by the addition of lead and arsenic to the raw material mixture, by the addition of a small amount of Sb<sub>2</sub>O<sub>5</sub> to the finished phosphor.

EXAMPLE III.—MAGNESIUM TUNGSTATE

70 In this test a mixture of MgO and WO<sub>3</sub>, in the proportion of 1.46 mols of MgO as basic carbonate per mol of WO<sub>3</sub>, was fired for about 6 hours at about 1900° F. The suspension of this fired material was prepared in substantially the same way as the suspension in Example I and

about .05%  $Sb_2O_3$  by weight of the finished phosphor was added thereto. The effect which the addition of  $Sb_2O_3$  had on the lumen maintenance and the brightness of 40 watt lamps coated with this suspension is indicated in the following table:

## LUMENS PER WATT

|                | 0<br>Hrs. | 100<br>Hrs. | 500<br>Hrs. |
|----------------|-----------|-------------|-------------|
| 0% $Sb_2O_3$   | 51.2      | 47.2        | 42.6        |
| .05% $Sb_2O_3$ | 50.6      | 48.0        | 44.4        |

Thus it may be seen that the addition of .05%  $Sb_2O_3$  to a suspension of magnesium tungstate enhances the lumen maintenance and the brightness of the fluorescent lamp.

## EXAMPLE IV.—BARIUM LEAD SILICATE

In this test a mixture of about 1 mol of  $BaCO_3$ , about 1.62 mols of  $SiO_2$  and about 0.12 mol of an activator,  $PbCO_3$ , was ball-milled in water, dried, crushed and fired for about 2 to 6 hours at about 1850° F. The suspension of this fired material was prepared in substantially the same way as the suspension in Example I and about .05%  $Sb_2O_3$  by weight of the finished phosphor was added thereto. The effect which the addition of  $Sb_2O_3$  had on the lumen maintenance of 20 watt lamps coated with this suspension is indicated in the following tables:

## LUMENS PER WATT

|                | 0<br>Hrs. | 100<br>Hrs. | 300<br>Hrs. | 500<br>Hrs. | 900<br>Hrs. |
|----------------|-----------|-------------|-------------|-------------|-------------|
| 0% $Sb_2O_3$   | 20.5      | 16.6        | 15.3        | 15.0        | 13.5        |
| .05% $Sb_2O_3$ | 19.8      | 17.6        | 16.5        | 16.3        | 14.9        |

Thus it may be seen that the addition of the  $Sb_2O_3$  to a suspension of barium silicate decreases the rate of loss in lumen maintenance and increases the brightness during the life of the lamp.

## EXAMPLE V.—CALCIUM LEAD MANGANESE SILICATE - MAGNESIUM TUNGSTATE BLEND

Tests were run on various blends of calcium lead manganese silicate and magnesium tungstate which are used to give white and daylight fluorescent lamps. The calcium lead silicate component was prepared by mixing about 1 mol of  $CaCO_3$ , about 1.2 mols of  $SiO_2$ , about 0.066 mol of an activator,  $MnCO_3$  and about 0.0035 mol of  $PbF_2$ , which in this case serves as an activator and a fluxing agent. This mixture was ball-milled in water, dried, crushed and fired for about 6 hrs. at about 1900° F. and again for about 6 hours at about 2100° F. This component was then mixed in the desired proportion with magnesium tungstate which was prepared substantially as indicated above in Example III.

Three tests were run, one with a daylight blend and two with a white blend. In the daylight test and in one of the white tests, .05% antimony in the form of the free metal was added to the suspension in some cases, and in other cases .05%  $Sb_2O_3$  was added, both of these percentages being by weight of the finished phosphor. Forty watt lamps were employed in these tests.

## LUMENS PER WATT

| Test I.—White Blend |  | 0<br>Hrs. | 100<br>Hrs. | 280<br>Hrs. | 498<br>Hrs. |
|---------------------|--|-----------|-------------|-------------|-------------|
| 0% $Sb_2O_3$        |  | 53.4      | 49.6        | 47.0        | 45.4        |
| .05% $Sb_2O_3$      |  | 51.8      | 50.2        | 48.2        | 48.2        |

| Test II.—White Blend |  | 0<br>Hrs. | 100<br>Hrs. | 296<br>Hrs. | 496<br>Hrs. |
|----------------------|--|-----------|-------------|-------------|-------------|
| 0% $Sb_2O_3$         |  | 52.0      | 51.0        | 48.8        | 47.8        |
| .05% $Sb_2O_3$       |  | 50.8      | 50.8        | 49.6        | 48.6        |
| .05% Antimony Metal  |  | 51.6      | 51.0        | 48.6        | 48.2        |

| Test III.—Daylight Blend |  | 0<br>Hrs. | 100<br>Hrs. | 333<br>Hrs. | 491<br>Hrs. |
|--------------------------|--|-----------|-------------|-------------|-------------|
| 0% $Sb_2O_3$             |  | 50.4      | 48.0        | 46.4        | 45.2        |
| .05% $Sb_2O_3$           |  | 49.6      | 49.4        | 48.0        | 47.0        |
| .05% Antimony Metal      |  | 49.6      | 49.4        | 48.2        | 47.4        |

These tests indicate that the addition of antimony, either in the form of the free metal or the trioxide, to the suspension of a blend of magnesium tungstate and calcium lead manganese silicate enhances the lumen maintenance and the brightness of the lamps.

## EXAMPLE VI—ZINC BERYLLIUM MANGANESE SILICATE-MAGNESIUM TUNGSTATE BLEND

These two materials were prepared in substantially the same manner and the several ingredients thereof were present in substantially the same proportions as indicated in Examples I and III above, and the fired powders were then blended in proportions to give a white lamp.

In Test I below, various amounts of  $Sb_2O_3$  were added to the suspension of this blend and 40 watt fluorescent lamps were made.

## LUMENS PER WATT

| Test I          |  | 0<br>Hrs. | 115<br>Hrs. | 312<br>Hrs. | 529<br>Hrs. | 852<br>Hrs. |
|-----------------|--|-----------|-------------|-------------|-------------|-------------|
| 0% $Sb_2O_3$    |  | 67.4      | 60.2        | 56.0        | 53.4        | 50.4        |
| .005% $Sb_2O_3$ |  | 67.4      | 61.6        | 58.2        | 55.2        | 52.0        |
| .05% $Sb_2O_3$  |  | 64.8      | 62.2        | 58.8        | 57.2        | 54.8        |
| .5% $Sb_2O_3$   |  | 58.6      | 56.8        | 56.6        | 56.2        | 54.0        |

This test indicates that, even when amounts as small as .005% are added, the lumen maintenance and the brightness is improved.

## Test II

In this test the blend was substantially the same except that the zinc beryllium magnesite silicate was prepared as in Example II above. Various amounts of  $Sb_2O_3$  based on the weight of the finished phosphor were added to the suspension of this blend and 40 watt lamps were made therefrom.

## LUMENS PER WATT

|               |  | 0<br>Hrs. | 121<br>Hrs. | 343<br>Hrs. | 502<br>Hrs. | 886<br>Hrs. | 1754<br>Hrs. | 2501<br>Hrs. |
|---------------|--|-----------|-------------|-------------|-------------|-------------|--------------|--------------|
| 0% $Sb_2O_3$  |  | 60.0      | 56.8        | 55.0        | 52.8        | 51.2        | 47.8         | 46.2         |
| .1% $Sb_2O_3$ |  | 59.4      | 58.4        | 57.6        | 56.0        | 55.4        | 52.8         | 51.0         |
| .2% $Sb_2O_3$ |  | 59.2      | 58.4        | 58.0        | 56.2        | 55.6        | 52.6         | 51.4         |
| .3% $Sb_2O_3$ |  | 58.8      | 58.2        | 57.6        | 55.6        | 55.0        | 53.2         | 52.0         |

This test indicates that as much as .3%  $Sb_2O_3$  can be employed with beneficial results both on the lumen maintenance and on the brightness during life.

7  
Test III

In this test the same fluorescent material blend was used as used in Test II immediately above. In this case, however, various amounts of the free metal were added to the suspension based on the weight of the finished phosphor, with the following results:

## LUMENS PER WATT

|                                     | 0<br>Hrs. | 98<br>Hrs. | 318<br>Hrs. | 498<br>Hrs. | 878<br>Hrs. |
|-------------------------------------|-----------|------------|-------------|-------------|-------------|
| No antimony                         | 64.4      | 58.6       | 56.4        | 55.0        | 53.2        |
| .05% Sb <sub>2</sub> O <sub>3</sub> | 63.2      | 61.0       | 59.0        | 58.3        | 56.0        |
| .05% Sb                             | 63.6      | 62.4       | 59.2        | 58.9        | 56.2        |
| .1% Sb                              | 62.2      | 60.8       | 58.2        | 58.5        | 56.8        |
| .5% Sb                              | 60.2      | 59.8       | 57.2        | 57.1        | 56.0        |
| 1.0% Sb                             | 58.8      | 58.8       | 57.2        | 56.9        | 56.4        |

The results of this test indicate that the addition of various small amounts of antimony metal to the fluorescent material suspension has a beneficial effect on lumen maintenance comparable to the advantages obtained by adding Sb<sub>2</sub>O<sub>3</sub>.

## EXAMPLE VII—VARIOUS ANTIMONY COMPOUNDS ADDED TO BLEND OF ZINC BERYLLIUM MANGANESE SILICATE AND MAGNESIUM TUNGSTATE

In this test various antimony compounds were added to a suspension of zinc beryllium manganese silicate—magnesium tungstate blend and 40 watt white lamps were made. The zinc beryllium manganese silicate was substantially the same as that described in Example II above, and the magnesium tungstate was substantially the same as that described in Example III above. The quantity of the antimony compound in each case was based on the weight of the finished phosphor. The following results were obtained:

## LUMENS PER WATT

|                                                                    | 0<br>Hrs. | 134<br>Hrs. | 270<br>Hrs. |
|--------------------------------------------------------------------|-----------|-------------|-------------|
| Control                                                            | 64.0      | 57.0        | 55.0        |
| .05% Sb <sub>2</sub> O <sub>3</sub>                                | 63.2      | 60.8        | 59.2        |
| .05% Sb <sub>2</sub> S <sub>3</sub>                                | 63.0      | 60.8        | 59.4        |
| .1% Sb <sub>2</sub> S <sub>3</sub>                                 | 61.6      | 59.2        | 58.0        |
| .05% Sb <sub>2</sub> O <sub>5</sub>                                | 64.8      | 60.8        | 59.4        |
| .1% Sb <sub>2</sub> O <sub>5</sub>                                 | 64.8      | 59.6        | 58.2        |
| .05% K <sub>2</sub> SbC <sub>4</sub> H <sub>9</sub> O <sub>7</sub> | 64.8      | 59.2        | 58.0        |
| .1% K <sub>2</sub> SbC <sub>4</sub> H <sub>9</sub> O <sub>7</sub>  | 64.2      | 60.2        | 59.2        |
| .05% SbSe                                                          | 65.0      | 59.0        | 56.6        |
| .1% SbSe                                                           | 64.0      | 59.8        | 58.4        |

The results of this test indicate that several antimony compounds other than the oxides have a beneficial effect on the lumen maintenance and the brightness of fluorescent lamps, although any antimony compounds which react chemically with the fluorescent material should generally be avoided.

In all of the examples above, antimony or one of its compounds was added to the finished phosphor. However, as pointed out above, in the case of some fluorescent materials, the antimony or its compounds may be added to the unfired raw material mixture with beneficial results on the lumen maintenance.

## EXAMPLE VII—ANTIMONY OXIDES ADDED TO ZINC BERYLLIUM MANGANESE SILICATE UNFIRED RAW MATERIAL MIXTURE

In this test the zinc beryllium silicate was of the same type and was prepared in substantially the same manner as that of Example I above, except that various amounts of Sb<sub>2</sub>O<sub>5</sub> and

Sb<sub>2</sub>O<sub>5</sub> were added to the unfired raw material mixture. This test was made with 20 watt lamps.

## LUMENS PER WATT

|                                     | 0<br>Hrs. | 102<br>Hrs. | 315<br>Hrs. | 917<br>Hrs. |
|-------------------------------------|-----------|-------------|-------------|-------------|
| 0% Sb <sub>2</sub> O <sub>5</sub>   | 52.0      | 43.3        | 38.7        | 35.0        |
| .1% Sb <sub>2</sub> O <sub>5</sub>  | 52.5      | 47.6        | 45.3        | 42.0        |
| .4% Sb <sub>2</sub> O <sub>5</sub>  | 48.2      | 45.2        | 43.8        | 41.6        |
| .8% Sb <sub>2</sub> O <sub>5</sub>  | 47.9      | 45.6        | 43.6        | 40.8        |
| 1.2% Sb <sub>2</sub> O <sub>5</sub> | 53.0      | 50.5        | 48.3        | 45.1        |

This test indicates that when various amounts of an oxide of antimony are added to the unfired raw material mixture, the lumen maintenance and the brightness are beneficially affected.

## EXAMPLE IX—ANTIMONY TRIOXIDE ADDITION TO MAGNESIUM TUNGSTATE UNFIRED RAW MATERIAL MIXTURE

Example III above shows that the addition of Sb<sub>2</sub>O<sub>3</sub> to the coating suspension of magnesium tungstate improved the lumen maintenance and brightness. However, the reverse is true when

Sb<sub>2</sub>O<sub>3</sub> is added to the unfired raw material mixture. Even a very small amount of Sb<sub>2</sub>O<sub>3</sub> introduced at this point seriously reduces the lumen maintenance and brightness as shown in the following table:

## LUMENS PER WATT

| Percent Sb <sub>2</sub> O <sub>3</sub> | 0<br>Hrs. | 98<br>Hrs. | 288<br>Hrs. |
|----------------------------------------|-----------|------------|-------------|
| 0.0000                                 | 51.2      | 47.2       | 46.2        |
| 0.0052                                 | 48.6      | 43.4       | 41.2        |
| 0.0100                                 | 47.0      | 42.0       | 39.8        |
| 0.0300                                 | 42.0      | 38.8       | 36.2        |
| 0.0518                                 | 40.8      | 36.4       | 35.0        |
| 0.5180                                 | 30.8      | 27.2       | 25.6        |

The amount of antimony is expressed in percent of tungstic oxide (WO<sub>3</sub>).

The effect of adding Sb<sub>2</sub>O<sub>3</sub> to the unfired raw material mixture of magnesium tungstate is thus opposite to the effect obtained by adding Sb<sub>2</sub>O<sub>3</sub> to the unfired raw material mixture of zinc beryllium manganese silicate (Example VIII above).

## EXAMPLE X—ADDITION OF ANTIMONY OXIDES TO ZINC BERYLLIUM MANGANESE SILICATE UNFIRED RAW MATERIAL MIXTURE AND TO FINISHED PHOSPHOR

Two tests were run with 20 watt lamps to determine the effect which the addition of antimony oxides to the raw material mixture and the finished phosphor had on the lumen maintenance as compared to antimony oxide additions to the raw material mixture only. The fluorescent material employed in these tests was substantially the same as that described in Example I above. In Test I, .05% Sb<sub>2</sub>O<sub>5</sub> was added to the raw material mixture and .05% Sb<sub>2</sub>O<sub>3</sub> was added to the finished phosphor in the case of the "test" lamps, whereas the "control" lamps had .05% Sb<sub>2</sub>O<sub>5</sub> added to the raw material mixture only.

## LUMENS PER WATT

| Test I  | 0<br>Hrs. | 100<br>Hrs. | 200<br>Hrs. | 600<br>Hrs. | 880<br>Hrs. |
|---------|-----------|-------------|-------------|-------------|-------------|
| Test    | 51.3      | 49.0        | 48.7        | 47.2        | 46.6        |
| Control | 50.0      | 46.9        | 44.0        | 41.7        | 39.8        |

In Test II, .05% Sb<sub>2</sub>O<sub>5</sub> was added to the raw material mixture and .05% Sb<sub>2</sub>O<sub>3</sub> was added to the finished phosphor in the case of the "test"

lamps, whereas the "control" lamps had .05% Sb<sub>2</sub>O<sub>5</sub> added to the raw material mixture only.

| Test II      | 0 Hrs. | 100 Hrs. | 300 Hrs. | 600 Hrs. | 880 Hrs. |
|--------------|--------|----------|----------|----------|----------|
| Test.....    | 54.7   | 53.2     | 50.5     | 49.6     | 47.8     |
| Control..... | 52.4   | 49.7     | 47.8     | 45.0     | 43.6     |

Thus these two tests indicate that when a small amount of an oxide of antimony is added to a finished phosphor which already contains a small amount of an oxide antimony, a further gain in L. P. W. maintenance is obtained.

In all of the above examples and tests, the envelope of the fluorescent lamps was a soda-lime glass. As pointed out above, the addition of antimony or certain compounds thereof is beneficial not only on the maintenance of the radiant flux output and brightness during life of fluorescent lamps but on other electric gaseous discharge devices, which contain a small quantity of a metal vapor such as mercury. The addition of antimony or certain compounds thereof to a germicidal lamp improves the maintenance of the radiant flux output thereof tremendously. The germicidal lamps on which the tests below were made was substantially the same as the lamp shown in Figure 1, except that the lamp envelope was a borosilicate glass substantially free of iron and designed to transmit germicidal ultra-violet radiations and the lamp envelope did not have a fluorescent coating thereon. Since germicidal lamps are used extensively in refrigerators, Test I below was made at 32° F. Test II was made at 80° F. In each test, the lamp envelope was coated with a mixture of 0.05 gram Sb<sub>2</sub>O<sub>3</sub> per c. c. of a lacquer such as nitrocellulose, and the envelope was heated to burn off the lacquer. The lamp was then processed in the conventional manner. The measurement of the radiant flux output in the tables below is in arbitrary relative units.

#### EXAMPLE XI.—GERMICIDAL LAMPS

| Test I, 32° F. | Control | Test |
|----------------|---------|------|
| hours          |         |      |
| 100.....       | 58.6    | 64.2 |
| 300.....       | 41.0    | 54.0 |
| 500.....       | 27.6    | 46.0 |

| Test II, 80° F. | Control | Test |
|-----------------|---------|------|
| hours           |         |      |
| 100.....        | 73.0    | 76.0 |
| 300.....        | 68.3    | 70.8 |
| 500.....        | 66.7    | 70.0 |

Thus by providing the borosilicate glass envelope of a germicidal lamp with a surface high in Sb<sub>2</sub>O<sub>3</sub> content the maintenance of the radiant flux output of the lamp is enhanced considerably, regardless of the ambient temperature conditions under which the lamp is operated.

In the several examples above, we have shown that the addition of a small quantity of antimony in the form of the free metal or certain of its compounds, enhances the maintenance of the radiant flux output of electric gaseous discharge devices. We have indicated various methods which may be employed in introducing the antimony or its compounds into the discharge devices. In the case of fluorescent lamps, when the antimony or its compounds is added to the

finished phosphor, to the suspension thereof, for example, we have indicated in each case, the quantity of the antimony or its compound which is added at this point. As was pointed out above, after the lamp envelope is coated, the envelope is heated to a temperature of about 450° C. to about 550° C. Analyses of the fluorescent coating in the finished lamp indicate that some of the antimony or its compound which was added to the finished phosphor is lost, probably due to the baking. For example, when about .05% of an oxide of antimony based on the weight of the finished phosphor is added thereto, only about .015% of antimony is left in the fluorescent coating in the finished lamp. When between .005% to 0.1% of an oxide of antimony is added to the finished phosphor, the amount of antimony which is left in the fluorescent coating in the finished lamp is between about .0015% to about .03%.

Unlike some other metals or oxides, antimony oxides in the amounts used herein do not appear to affect the coating adherence, neither increasing nor decreasing it. When antimony metal is added to the suspension, it is probably oxidized, at least in part, during the baking process.

Putting the antimony in the final phosphor suspension appears to be helpful with all fluorescent materials, excepting possibly those with which it might chemically react, and can therefore be used even with those phosphors which it adversely affects if used in the unfired raw material mix. The beneficial action of the antimony appears to be with the glass or the discharge, and not directly on the phosphor.

What we claim is:

1. A fluorescent lamp comprising a glass envelope, electrodes sealed in said envelope, a filling of at least one inert gas at low pressure in said envelope, a quantity of mercury in said envelope, and a coating on the inside wall of said envelope, said coating comprising an activated fluorescent material and about 0.015% antimony in the oxide form.
2. A fluorescent lamp comprising a glass envelope, electrodes sealed in said envelope, a filling of at least one inert gas at low pressure in said envelope, a quantity of mercury in said envelope, and a coating on the inside wall of said envelope, said coating comprising an activated fluorescent material and between about 0.0015% to about 0.03% antimony in the oxide form.

JOSEPH ARTHUR ROY.  
ROBERT S. IVES.

#### REFERENCES CITED

The following references are of record in the file of this patent:

#### UNITED STATES PATENTS

| Number       | Name       | Date          |
|--------------|------------|---------------|
| 60 2,177,691 | Dawihl     | Oct. 31, 1939 |
| 2,241,950    | Huniger    | May 13, 1941  |
| 2,306,626    | Huniger    | Dec. 29, 1942 |
| 2,316,366    | Ruttenauer | Apr. 13, 1943 |
| 65 2,317,977 | Casellini  | May 4, 1943   |
| 2,344,081    | Claude     | Mar. 14, 1944 |
| 2,433,404    | Smith      | Dec. 30, 1947 |

#### FOREIGN PATENTS

| Number     | Country       | Date          |
|------------|---------------|---------------|
| 70 578,195 | Great Britain | June 19, 1946 |

#### OTHER REFERENCES

Webster's New International Dictionary (2nd ed.) 1934, pg. 1062, Merriam-Webster, Springfield, Mass.